

Patented Aug. 14, 1945

2,381,868

# UNITED STATES PATENT OFFICE

2,381,868

## TEXTILE PRINTING COMPOSITIONS

John R. Abrams, Jersey City, N. J., assignor to  
Interchemical Corporation, New York, N. Y., a  
corporation of Ohio

No Drawing. Application May 1, 1941,  
Serial No. 391,343

4 Claims. (Cl. 260—24)

This invention relates to compositions for use in textile decorating with pigments, and is directed particularly to such compositions in which the pigment binder comprises a carbamide-formaldehyde resin and methyl abietate.

Conventional textile printing is ordinarily done with water solutions of dyestuffs containing water-soluble thickening agents in sufficient quantity to retard the spreading of the color on the fabric after printing. The dyestuff is fixed onto the fabric by some chemical process, and the thickening agent is then washed out of the fabric. The time and expense involved in this after-treatment, added to the originally high color cost for light and tub-fast dyes, has been a major problem in textile printing. An unsolved problem has been the reproduction of very fine designs. Since the pastes spread on the fabric after printing when thin enough to be removed sharply from fine engravings, giving blurred designs, it has been found impossible to use photogravure cylinders or extremely fine mill and dye engravings. Attempts to modify these pastes by addition of wetting agents and emulsification of oils therein have not solved the basic difficulties.

The use as printing pastes of colored lacquers (which, for the purpose of this application are defined as dispersions of color in vehicles consisting of a solution of a plastic or solid film-forming, water-resistant binder such as a cellulose derivative or a resin, in an organic solvent or mixture of solvents) has been attempted in order to overcome the difficulties with prior art pastes, but has not been successful commercially. Relatively few lacquer compositions withstand both dry cleaning and washing; and such compositions as are resistant have been generally unacceptable due to the fact that the fabrics, when printed with these lacquers, develop an undesirable stiff feel (known to the trade as "hand"), to the necessity for using large amounts of color to obtain deep shades, and to the tendency of colored markings to rub off onto other clothing and leave a mark (known as "crocking").

In the Jenett U. S. Patent No. 2,222,581, issued November 19, 1940, there is described a new type of textile printing paste which eliminates the disadvantages of the conventional dye printing pastes and avoids the difficulties which have been encountered in the prior art lacquer printing pastes. These pastes are emulsions in which an outer continuous water-immiscible lacquer phase is thickened by an inner aqueous

phase which is at least 20 per cent. of the total emulsion, by weight. Preferably, the binder of the lacquer is one which is originally soluble in ordinary organic solvents and which can be converted into an insoluble state after printing—most desirably, a readily heat-polymerizable synthetic resin, best exemplified by the plasticized urea formaldehyde resins.

The use of pastes made in accordance with this patent permits of the use of cheap pigments and avoids the after-treatment necessary with conventional printing pastes. The pastes separate sharply even from very fine photogravure cylinders, although thickened sufficiently to prevent any spreading on the fabric; this makes possible much finer printing than can be obtained with conventional pastes. The hand imparted to fabrics by these pastes is very much less than the hand imparted to similar fabrics by ordinary lacquer pastes having the same binder, the amount of color needed to produce deep shades is sharply reduced, and the crocking substantially eliminated.

I have discovered that improved results can be obtained in pastes of this type, particularly with respect to wash-fastness, by using as the binder a carbamide-formaldehyde resin in the solvent-soluble state and the methyl ester of abietic acid.

In general, I use from 1 to 4 parts by weight of resin to 1 part by weight of methyl abietate; all compositions in this range give acceptable prints which are superior in wash-fastness to combinations of urea formaldehyde and alkyd resins. The optimum wash-fastness is obtained with from 2 to 3 parts of resin per part of methyl abietate.

I do not know why such superior wash-fastness is obtained by the use of this ester as a plasticizer, since abietic acid, and abietic acid alkyd resins, are not as good when used with carbamide-formaldehyde resin, as ordinary oil-modified alkyd resins in this respect.

This type of emulsion paste, while intended primarily for printing, may be used for dyeing by immersing the cloth in the emulsion paste, and forcing the paste through the cloth by mechanical or other action. When so used, the resin-pigment complex does not saturate the fabric, but on microscopic examination is found as isolated islands spaced in such fashion that a full color effect is given to the unaided eye. Hence, the fabric remains completely pervious to washing as when the composition is printed, and the fibers are not matted together as in ordinary

impregnations. This discontinuity of film in both printing and dyeing serves to distinguish this type of fabric treatment from ordinary fabric coating.

Typical examples of my invention are the following:

*Example 1*

|                                              | Parts by weight |
|----------------------------------------------|-----------------|
| 50% solution of urea formaldehyde resin in   | 10              |
| 30 butanol, 20 xylene                        | 20.0            |
| Methyl abietate                              | 5.0             |
| Pine oil                                     | 6.6             |
| Solvesso #2 (hydrogenated petroleum naphtha) | 15.4            |

are mixed, and a mixture of—

|                                         | Parts by weight |
|-----------------------------------------|-----------------|
| A 23% aqueous phthalocyanine green pulp | 13.0            |
| A 8.5% aqueous bentonite dispersion     | 17.7            |
| Water                                   | 22.3            |

is added slowly to the organic mixture, with stirring. The complete mixture is passed through a colloid mill, and gives a smooth water-in-lacquer emulsion.

When printed or padded onto fabric, it can be set by heating for several minutes at 250° F., or for some seconds at 300° F.; the resultant print is unusually wash-fast.

*Example 2*

|                                         | Parts by weight |
|-----------------------------------------|-----------------|
| Urea resin solution of Example 1        | 22.50           |
| Methyl abietate                         | 3.75            |
| Pine oil                                | 6.20            |
| Solvesso #3                             | 14.55           |
| Indanthrene Blue GGSNL, 15% water paste | 20.00           |
| Bentonite dispersion—85%                | 17.70           |
| Water                                   | 15.30           |

*Example 3*

|                                                                               | Parts by weight |
|-------------------------------------------------------------------------------|-----------------|
| Melamac 245-8 (50% solution of melamine-formaldehyde resin in butanol-xylene) | 20.0            |
| Methyl abietate                                                               | 5.0             |
| Pine oil                                                                      | 5.0             |
| Turpentine                                                                    | 13.0            |
| Copper phthalocyanine blue, 20% water pulp                                    | 7.5             |
| Water                                                                         | 49.5            |

CERTIFICATE OF CORRECTION.

Patent No. 2,381,868.

JOHN R. ABRAMS.

August 14, 1945.

It is hereby certified that error appears in the printed specification of the above numbered patent requiring correction as follows: Page 2, first column, line 39, Example 2, for "85%" read --8.5%--; page 2, second column, line 11, Example 3, for that portion of the formula reading "X-C" read --X=C--; and that the said Letters Patent should be read with this correction therein that the same may conform to the record of the case in the Patent Office.

Signed and sealed this 25th day of December, A. D. 1945.

Leslie Frazer

First Assistant Commissioner of Patents.

(Seal)

impregnations. This discontinuity of film in both printing and dyeing serves to distinguish this type of fabric treatment from ordinary fabric coating.

Typical examples of my invention are the following:

*Example 1*

|                                              | Parts by weight |
|----------------------------------------------|-----------------|
| 50% solution of urea formaldehyde resin in   | 10              |
| 30 butanol, 20 xylene                        | 20.0            |
| Methyl abietate                              | 5.0             |
| Pine oil                                     | 6.6             |
| Solvesso #2 (hydrogenated petroleum naphtha) | 15.4            |

are mixed, and a mixture of—

|                                         | Parts by weight |
|-----------------------------------------|-----------------|
| A 23% aqueous phthalocyanine green pulp | 13.0            |
| A 8.5% aqueous bentonite dispersion     | 17.7            |
| Water                                   | 22.3            |

is added slowly to the organic mixture, with stirring. The complete mixture is passed through a colloid mill, and gives a smooth water-in-lacquer emulsion.

When printed or padded onto fabric, it can be set by heating for several minutes at 250° F., or for some seconds at 300° F.; the resultant print is unusually wash-fast.

*Example 2*

|                                         | Parts by weight |
|-----------------------------------------|-----------------|
| Urea resin solution of Example 1        | 22.50           |
| Methyl abietate                         | 3.75            |
| Pine oil                                | 6.20            |
| Solvesso #3                             | 14.55           |
| Indanthrene Blue GGSNL, 15% water paste | 20.00           |
| Bentonite dispersion—85%                | 17.70           |
| Water                                   | 15.30           |

*Example 3*

|                                                                               | Parts by weight |
|-------------------------------------------------------------------------------|-----------------|
| Melamac 245-8 (50% solution of melamine-formaldehyde resin in butanol-xylene) | 20.0            |
| Methyl abietate                                                               | 5.0             |
| Pine oil                                                                      | 5.0             |
| Turpentine                                                                    | 13.0            |
| Copper phthalocyanine blue, 20% water pulp                                    | 7.5             |
| Water                                                                         | 49.5            |

CERTIFICATE OF CORRECTION.

Patent No. 2,381,868.

JOHN R. ABRAMS.

August 14, 1945.

It is hereby certified that error appears in the printed specification of the above numbered patent requiring correction as follows: Page 2, first column, line 39, Example 2, for "85%" read --8.5%--; page 2, second column, line 11, Example 3, for that portion of the formula reading "X-C" read --X=C--; and that the said Letters Patent should be read with this correction therein that the same may conform to the record of the case in the Patent Office.

Signed and sealed this 25th day of December, A. D. 1945.

Leslie Frazer

First Assistant Commissioner of Patents.

(Seal)